

## UNITED STATES PATENT OFFICE.

HANS T. CLARKE AND CARL J. MALM, OF ROCHESTER, NEW YORK, ASSIGNORS TO EASTMAN KODAK COMPANY, OF ROCHESTER, NEW YORK, A CORPORATION OF NEW YORK.

## PROCESS OF ESTERIFYING MERCERIZED CELLULOSE WITH LOWER FATTY ACIDS.

No Drawing.

Application filed April 23, 1927. Serial No. 186,170.

This invention relates to processes of esterifying mercerized cellulose with lower fatty acids, preferably those containing more than 1 and less than 8 carbon atoms.

- 5 **5** One object of our invention is to provide an inexpensive and simple process of producing cellulose esters of the lower fatty acids without the aid of anhydrides or catalysts. Another object of the invention is 10 to provide a process of making cellulose esters of the lower fatty acids in a plurality of stages, certain of the acid groups being combined into the ester during the first stage without use of anhydrides and catalysts, and 15 the remainder of the acid groups being combined in the ester by the subsequent treatment of the esters formed in the first stage, thus effecting an economy in expensive ingredients, such as the anhydrides of the acids. 20 Another object of the invention is to provide a process in which the first-stage esterification is performed in the absence of any material more hydrolytic than the fatty acids themselves, thus leaving the cellulosic material with the minimum molecular degradation and essentially unchanged in its physical appearance by the first stage of the process. Other objects will hereinafter appear.

In our application, Serial No. 122,028, 30 filed July 12th, 1926 for "cellulose esters of fatty acids and processes of making the same" we have shown that unmodified or undegraded cellulose can be esterified, under proper conditions, by the lower fatty acids 35 without the use of catalysts or expensive anhydrides and the like. In the case of each of the lower fatty acids, approximately one molecular proportion of acid is combined with an amount of cellulose corresponding to 40 24 carbon atoms. This first-stage ester is then esterified further by the usual process, but with notable economies in the use of anhydrides and with mild catalysts to avoid molecular degradation.

45 We have now found that cellulose esters of the lower fatty acids may be prepared in which more than 2 molecular proportions of acid are combined with an amount of cellulose corresponding to 24 carbon atoms and 50 without the use of anhydrides or catalysts,—

in fact, with the minimum molecular degradation and without modifying the physical appearance of the treated cellulosic material. We are able to bring about this result by first mercerizing the cellulosic raw 55 material before it is heated with the acid as the sole acylating agent. These first-stage esters prepared by simple heating of the mercerized cellulose with the acids as the sole acylating agents are very stable, as indicated 60 by their resistance to splitting off acetyl groups when tested by prolonged boiling in water. In general the fibers of the new compounds are superficially indistinguishable 65 from the mercerized cellulose fibers from which they are prepared.

It is a useful fact that these esters are more readily esterified than plain cellulose or mercerized cellulose fibers. Moreover, it is necessary to add fewer acetyl groups to 70 them, since they already contain useful amounts. The practical effect is that when these esters are further esterified by using anhydrides, or even acyl chlorides, in the ways previously described for the acylation of 75 cellulose itself, savings of from 20 to 40% of the amount of anhydrid or chlorid may be obtained. A substantial saving is effected so long as our first-stage esters have more than one acyl group for each 24 carbon atoms 80 in the cellulose.

Our invention is concerned with the esters of the fatty acids having more than 1 and less than 8 carbon atoms, such as acetic, propionic, butyric, valeric, caproic, 85 heptylic, etc. The rate of esterification falls off rapidly with the higher members of this series of acids. Consequently acetic acid, propionic acid and butyric acid are those which are preferred, because of their 90 relatively greater commercial availability and their greater speed of reaction. Acetic acid is commercially the most important at present, because of its lower cost.

For the raw cellulose to be mercerized we 95 can employ any of the types customarily used in the manufacture of esters such, for instance, as cotton, surgical cotton, wool, tissue paper especially prepared from cotton, and even sulfite wood pulp, (preferably 100

bleached). Our process has a notable whitening tendency on the cellulose where the latter is initially colored, but the general appearance of the fibers is not changed. In other words, they do not swell, gelatinize, or go into solution during the treatment with the fatty acids in the first stage.

The first-stage esterification may be conducted over a considerable temperature range. In general we prefer to operate above 100° C. in order to insure reasonably rapid action and we do not advise the use of temperatures above 170° C., because of the danger of molecularly degrading the cellulose and the products produced from it. Within this preferred range the temperatures vary with the boiling points of the different acids. For example, those acids which boil below 170° C. can be used at atmospheric pressure, a considerable excess of acid over the amount which will enter the ester being used. But we find that the time can be very considerably shortened by using a superatmospheric pressure, say in an autoclave, provided the corresponding temperature does not reach the point where the product is degraded. While we use the acids as the sole acylating agents and prefer to employ them without admixture with other liquids, nevertheless, the esterification can be effected, when the acids are mixed with non-acylating liquids, such as chloroform, carbon tetrachloride or benzene. But these produce no marked advantage.

During the first-stage acylation it is desirable to keep the amount of water present very low. The total water present, including the water in the original ingredients, plus the water formed during the esterification, should never be allowed to reach the point where it prevents the introduction of more than 8% of the acyl group. We aim to maintain the conditions during the reaction such that the water is removed or diminished in quantity. The use of a fractionating column is one way of obtaining this result, the water vapor being allowed to pass out while the fatty acids are condensed and flow back to the bath. This is possible because all of the fatty acids having more than 1 and less than 8 carbon atoms boil considerably above the boiling point of water.

The mercerization pretreatment of the cellulose is along customary lines. For example, the mercerization may be conducted at room temperature, by simply immersing the cellulose fibers in a dilute solution of alkali, such as sodium hydroxid. The time of mercerization, known as "aging" will be longer the more dilute the bath. With an 18% aqueous sodium hydroxid solution, we have obtained satisfactory results upon stopping the mercerization at the end of 24 hours, but no harm results when the mer-

cerization in such a solution has been carried out for over 72 hours,—48 hours being a good medium time. Moreover, a mercerization in a 40% aqueous solution of sodium hydroxid for 24 hours is effective and without harm to the molecule. After soaking in the alkaline solution, the latter is drained off and the mercerized cellulose fibers washed free from alkali with water and dried in the air at 30 to 40° C.

If desired, the water may be removed by washing with a suitable organic liquid miscible with water, such as alcohol or acetone, previous to drying. Acetic acid may be employed, in which case air-drying is rendered unnecessary. The water may also be removed by distillation with a water-immiscible liquid of suitable boiling temperature, such as benzene or carbon tetrachloride.

In the first stage of esterification the mercerized cellulose, thus prepared, is heated in the acid until the acetyl group introduced in the ester is at least 8% of the latter. For example, we may boil 1 part by weight of the mercerized cellulose in an excess of acetic acid, say 30 to 40 parts by weight, the operation being carried out at atmospheric pressure. The acid is initially substantially free from water, say of 99 to 100% strength. The boiling point of the reaction bath is thus kept at about 117° C. or slightly above. Of course, any suitable precautions are taken to prevent the loss of acid by loss of its vapors, the same being condensed and returned to the bath by the use of any of the expedients familiar to chemists.

As the boiling in acetic acid is continued under these conditions the esterification progressively takes place. Roughly the proportion of acetyl can be carried to well over 14% and even above 20% of the weight of the ester. This strong esterification may be obtained after different lengths of time, according to the method by which the cellulose was dried. Some of them reach approximately 14% after 96 hours of treatment. But a useful product is obtained after a much shorter time. For instance, the percentage of acetyl in the ester reaches 8% before 48 hours in practically every instance and often reaches 11% in that time. This 8% ester has the property of being readily esterified further in the usual baths but with very good economy in acetic anhydrid. It should be noted that in the above discussion, as well as in the claims, we have referred to the percentage of the acyl group, such as the acetyl group. The percentages thus given, correspond in each instance to a still higher percentage of "combined acid," the relation being in the proportion of the molecular weight of the acyl group to the molecular weight of the acid. For instance, 8% of the acetyl group means about 11.2% of combined acetic acid.

The following table illustrates the manner in which acetic acid reacts with cotton cellulose which has been mercerized, washed, and freed of water under different conditions:

5

*Times of boiling in acetic acid.*

| No. of experiment | Percentages of acetyl |         |         |          |          |          |          |
|-------------------|-----------------------|---------|---------|----------|----------|----------|----------|
|                   | 24 hrs.               | 48 hrs. | 96 hrs. | 200 hrs. | 300 hrs. | 400 hrs. | 500 hrs. |
| 10                |                       |         |         |          |          |          |          |
| 1                 | 7.4                   | 8.5     | 11.0    | 11.6     | 12.9     | 14.1     |          |
| 2                 | 7.7                   | 9.3     | 11.9    | 12.3     | 14.5     | 15.9     |          |
| 3                 | 9.3                   | 11.6    | 13.5    | 17.5     | 19.2     | 20.9     |          |
| 4                 | 10.2                  | 13.0    | 14.8    | 17.6     | 19.5     | 22.2     | 22.6     |

- 15 In experiment No. 1 the mercerization had been done in an 18% NaOH solution for 48 hours at room temperature but it was dried after washing and before boiling in acid. In No. 2 a 40% solution of NaOH was 20 used in mercerizing the fibers being finally dried as in No. 1. But in Nos. 3 and 4 after mercerizing, in 18% and 40% NaOH solutions respectively, for 48 hours at room 25 temperature and washing out the free alkali, the water was removed from the fiber by repeated washing with glacial acetic acid. The mercerized fibers were then boiled in acid without having been dried. Since 30 No. 1 and No. 2 were exactly parallel with No. 3 and No. 4, except for the drying operation, it will be seen that the dehydration without drying greatly speeds up the process, even more than the use of a strong mercerizing solution, as in No. 2 and No. 4.
- 35 After this first-stage esterification, the excess of acid is removed if the ester is to be further esterified in a bath containing an anhydrid and a catalyst. Part of the acid can, however, be left with the ester to function 40 as a diluent or a solvent during the second stage acylation, as is usual in the ordinary acetylation of plain cellulose. If the acetylated fibers, from the first stage, are desired to be used in that condition, they 45 are, of course, thoroughly washed in water and dried, in which event they look like the mercerized fibers from which they were derived. Instead of the acetic acid in the 50 above example, we may employ equimolecular parts by weight of propionic or butyric acid and employ, preferably, a fractionating column through which the water vapors may 55 pass, while retaining the acid vapors. The time of boiling is conveniently about 200 hours.

When 30 parts of heptylic acid are used with 1 part by weight of mercerized cellulose, the temperature should be kept below 165° C. and preferably above 145° C. This is under the boiling point of the acid, but sufficient to obtain a useful esterification without degradation.

When it is desired to work at superatmospheric pressures, 1 part of mercerized

cellulose may be heated, for example, with 65 30 parts of acetic acid by weight of 99 to 100% strength at a temperature between 140 and 160° C., say in a vessel of the autoclave type. The time of esterification is enormously shortened under these conditions, 70 being generally less than 10 hours.

The esterification may even be carried out with the vapors of the acids. For example, the mercerized fibers may be placed in an acid-resisting tube heated by any suitable 75 means, such as an oil bath, and the vapor of acetic acid conducted through the tube. This operation may be conducted either at atmospheric pressure or subatmospheric pressure, provided the temperatures do not go above 80 170° C. The excess of acid vapor may be repassed or recirculated, preferably after slightly reheating, through the tube. This enables a rapid acetylation to take place. The subsequent esterification of the first-stage esters can take place in any of the usual esterifying baths, but with the amount of anhydrid diminished by from 20 to 40%. Moreover, the increased susceptibility of our 85 first-stage esters to further esterification 90 enables us to carry out the latter operation without the use of strong catalysts, thus avoiding the danger of degradation when such catalysts as sulfuric acid are employed. We can operate with a milder and safer one, 95 such as zinc chlorid or magnesium perchlorate trihydrate. As such esterification methods have been previously described, it is unnecessary to go over them in detail here.

Having thus described our invention, what 100 we claim as new and desire to secure by Letters Patent is:

1. In the process of making a cellulose ester of a fatty acid, mercerizing the cellulose and thereafter heating together the mercerized cellulose and a fatty acid having more than 1 and less than 8 carbon atoms without a catalyst at a temperature between 100° and 170° C. inclusive until the acyl group in the ester thus produced reaches at least 8%, said acid being the sole acylating agent. 105

2. In the process of making cellulose acetate, mercerizing the cellulose, and heating together the mercerized cellulose and substantially anhydrous acetic acid without a catalyst above 100° C. and below 170° C. inclusive until the acetyl group in the ester thus produced reaches at least 8%, said acetic acid being the sole acetylating agent. 115

3. In the process of making a fatty acid cellulose ester, mercerizing the cellulose, partially esterifying the mercerized cellulose with a fatty acid having more than 1 and less than 8 carbon atoms, in the absence of any anhydrid or catalyst, until there is more than one acyl group in the ester for each 24 carbon atoms in the cellulose, and 125

thereafter esterifying it further with the aid of an anhydrid of a fatty acid and a catalyst.

4. In the process of making a fatty acid cellulose ester, mercerizing the cellulose, heating the mercerized cellulose with a fatty acid having more than 1 and less than 8 carbon atoms without any catalyst until the acyl group in the ester thus formed reaches at least 8%, said acid being the sole acylating agent, and thereafter further esterifying it with the aid of an anhydrid of a fatty acid and a catalyst.

5. In the process of making cellulose acetate, mercerizing the cellulose, heating the cellulose in an excess of acetic acid at a temperature between 100° and 170° C. in the absence of a catalyst, the acid being the sole acetylating agent, until the acetyl group in the ester reaches at least 8%, and thereafter further acetylating the ester thus produced in the presence of acetic anhydrid and a milder catalyst than sulfuric acid.

6. In the process of making a cellulose ester of a fatty acid, mercerizing the cellulose in an aqueous alkaline solution, washing out the alkaline solution from the cellulose with water, removing the water from the cellulose with a substantially anhydrous organic liquid and heating the cellulose thus prepared with a fatty acid having more than

1 and less than 8 carbon atoms in the absence of a catalyst at a temperature between 100° and 170° C. inclusive until the acyl group from said acid in the ester thus produced reaches at least 8%.

7. In the process of making cellulose acetate, mercerizing the cellulose in an aqueous alkaline solution, washing out said solution with water, washing out the water with glacial acetic acid, boiling the cellulose in glacial acetic acid without a catalyst until the acetyl group in the ester thus produced reaches at least 8%, said acetic acid being the sole acetylating agent.

8. In the process of making a cellulose ester of a fatty acid, mercerizing the cellulose in an aqueous alkaline solution, dehydrating the cellulose with a substantially anhydrous organic liquid, and heating the cellulose thus prepared with a fatty acid, having more than 1 and less than 8 carbon atoms at a temperature between 100° and 170° C. inclusive in the absence of catalysts or anhydrides, until more than one acyl group is esterified with the cellulose for every 24 carbon atoms in the latter.

Signed at Rochester, New York, this 18th day of April, 1927.

HANS T. CLARK.  
CARL J. MALM.